

Feb. 10, 1931.

B. C. GOSS

1,792,010

GELATIN COMPOSITION CONTAINER

Filed April 24, 1929.



Inventor:  
Byron C. Goss,

by Joseph W. Harris

Atty.

## UNITED STATES PATENT OFFICE

BYRON C. GOSS, OF CLEVELAND, OHIO, ASSIGNOR TO THE LAKE ERIE CHEMICAL COMPANY, A CORPORATION OF OHIO

## GELATIN-COMPOSITION CONTAINER

Application filed April 24, 1929. Serial No. 357,770.

This invention relates to improvements in gelatin compositions, which may be used for lining receptacles, or for making capsules or containers or for similar uses.

5 An object of the invention is to provide a composition of organic matter which is relatively inexpensive, and which is comparatively soft, flexible, and resistant to the corroding action of a variety of chemical compounds.

10 A further object is to provide a container of organic matter which is sufficiently rigid at ordinary temperatures, to be safely handled, which is not brittle but which is destructible at higher temperatures, and which will not have a detrimental reaction upon, and accordingly will not spoil the contents of the container.

15 A further object is to provide a container of organic matter and a closure made of or coated with, the same material, which will prevent loss of its contents by leakage, etc.

20 A further object is to provide a container for "asphyxiating", or "tear" gas chemicals, the loaded container to be used in a cartridge, and capable of being discharged when "fired" in a pistol, the container and contents being ejected by propellant powder in the cartridge, the material of the container being of comparatively soft gelatinous organic matter, and which is shredded or destroyed by the firing of the cartridge, the parts of the container being incapable of injuring anyone when the cartridge is "fired" at close range 25 and parts of the container strike the person intended as the target.

25 A further object is to provide a container for chemicals to be used in cartridges and the like, the container being made of a corrosion resisting gelatinous substance that is comparatively soft and readily destroyed or shredded by the "firing" of the cartridge in a pistol.

40 A further object is to provide a composition of organic matter for containers to be used for asphyxiating gas chemicals, the composition being capable of resisting softening in humid atmospheres, and in hot weather, or 45 when carried on the person.

Other objects of the invention will appear to those skilled in this art.

In the accompanying drawing—

Fig. 1 represents a vertical section of a conventional type of container, with an inside fitting perforated cover just above, made of the gelatin corrosion resisting composition, the perforation being shown exaggerated in diameter for purposes of illustration;

Fig. 2 is a duplicate of Fig. 1, with the cover inserted, but not sealed;

Fig. 3 represents a composition container, similar to Figs. 1 and 2, containing a charge of chemicals, with the cover inserted, and the cover sealed thoroughly with the same or similar composition as that of which the container and cover are made, the sealing material also extending over the edges of the container.

Fig. 4 represents a vertical section of a conventional type of metal or fibrous container, coated inside and over the edges of the opening with the gelatin corrosion resisting composition, and a perforated metal cover just above, the cover also being coated with the composition;

Fig. 5 is a duplicate of Fig. 4 with the cover inserted, but not sealed;

Fig. 6 represents a vertical section of a metal container, coated inside with the gelatin corrosion resisting composition, and having a cover made of the composition, as in Figs. 1 and 2. This type of cartridge may be used instead of that shown in Fig. 7.

Fig. 7 represents a vertical section of a cartridge containing a gelatin composition shell filled with asphyxiating gas chemicals, and also a propellant powder charge, and a primer; and

Fig. 8 is a vertical section of a gelatinous composition container, with an outside fitting cover, instead of an inside fitting cover.

Gelatinous capsules as heretofore made, have not been practicable for use as containers for asphyxiating gas chemicals; the containers were too brittle for the service required, and had the property of softening in humid atmospheres and in hot weather, or in heated surroundings. A container to be practicable for this special service requires

a composition that will firmly adhere to and become integral with the sealing composition used therewith; it should not be brittle, otherwise cracks or fractures in its wall may result when it is sealed, or if it is roughly handled; it should be free from all tendency to soften as a result of hot or humid weather or surroundings. The sealing of the container is of considerable importance; care is required to avoid getting the molten sealing composition into the body of the chemicals.

The corrosion resisting gelatin composition of this invention is preferably made as follows:—

15 Weigh out one hundred and fifty (150) grams of high grade gelatin, for example No. 5-X sheet gelatin and place in a glass or enameled vessel of about six quarts capacity which has been about three-quarters filled 20 with water or a water solvent at 75° F. (24° C.). Let the sheet gelatin soak until it has taken up about one and one-half times its weight of water, about two hundred and twenty-five (225) grams, (the time required 25 is about 38 minutes). If desired, the water may contain some glycerine. Place the water soaked gelatin in a suitable heater, for example an electrically heated glue-pot, and turn on the current. When the gelatin has 30 melted, and is of a uniform consistency, add about fifty (50) grams of glycerine and stir thoroughly. The mixed mass should be maintained at about 170° F. (76.7° C.), and if it becomes too viscous, a small amount of water 35 at 75° F. may be added, (cold water should not be added). Only one heating of the gelatin mass should be made. If desired, suitable non-reacting colors may be dissolved in the melted mass, to produce capsules of different colors, in order that particular compositions may be placed in special containers. Or the gelatin mass used for the caps may alone be colored. The caps or closures 40 may if desired be made from an inferior grade of gelatin, such as a good grade of glue. The gelatin mass should preferably be used in a room at from 75° to 80° F., with very little drafts and with a relative humidity of 40%—55%. For different substances, 45 the quantity of glycerine added may vary from about nine percent to thirty-five percent, and of water, from fifty percent to about one hundred and fifty percent, of the weight of the gelatin used.

50 After the mass has been prepared as above described, it is formed into capsules 1, and caps 2, Fig. 1, by processes well known in the art, the caps are perforated at 3, with a needle, which may be heated if desired to 55 avoid any cracking of the material. The thickness of the walls on the drawing is exaggerated for purposes of illustration.

The capsules and caps are now carefully cleaned of all foreign matter. The following method of cleaning has been found to be

satisfactory. All surfaces which will be in contact with the chemicals to be placed in the containers are rubbed with a cloth saturated with carbon tetrachloride, particular care is taken to clean both sides of the caps, and the 70 inside of the capsules at least as far down as the caps extend.

The bodies of the capsules 1 are now placed upright in suitable trays, and filled to approximately eighty percent (80%) of their 75 capacity with one of the "asphyxiating" gas type of chemical compositions, 10, desired. As noted above, when desired, capsules of certain colors may be used for particular compositions. One of such compositions, so named Blind-X, made of chloracetophenone and ethylbromacetate, is poured into the cleaned capsules at room temperature, and the cleaned perforated caps applied. The cap is pressed down until the upper surface 85 is preferably just below the flush edges of the capsule. The filled capsule with the cap in place is now sealed, Fig. 3, by applying a quantity of the melted gelatin mass 11, as for example by pouring on top of, and around the joint, at the edges of the capsule, and over the perforation. Any bubbles arising should be wiped off before the gelatin seal sets. After the capsules have been sealed, 90 they should be allowed to stand for about thirty minutes, after which they may, if desired, be painted on the outside at 12 with the same sealing material. This outside painting may extend from the top down to a point just below where the cap extends within the 95 capsules, and tends to soften the capsule and helps to prevent fractures.

In the modifications shown in Figs. 4, 5, and 6, a suitable metal or fibrous container 4 is coated on the inside with gelatin, 5, the coating extending over the lip, at 6. The metal or fibrous cover, 7, is also coated on both sides, at 8 and 9, with the gelatin composition. The container is closed and sealed as described in connection with Fig. 3. 110

In Fig. 7, a charged and sealed gelatinous capsule, 15, containing a charge of asphyxiating gas chemicals 16, is placed in a cartridge shell 17, the latter containing the propellant powder charge 18, and a usual primer 19. When the cartridge is "fired" at a person from a pistol, the gelatinous composition of the capsule 15 is either destroyed, or is shredded into small fragments which are soft, and will not injure a person should the gelatinous fragments hit the victim in the face; the chemicals 16 will, however, be converted into a mass of gaseous asphyxiating fumes which are projected as a blast and will overcome the victim, rendering his capture easy, 115 and without doing permanent physical injury.

In Fig. 8, the cap 20 fits tightly on the outside of the capsule 21, and after filling, may be sealed by first applying a thick coat of the 120

molten gelatinous composition as a paint to the inside edge of the cap, and then quickly applying the cap; the molten gelatinous mass cementing the cap to the body of the capsule, 5 after which the hole 22 in the top of the cap is also sealed as described above.

The filled and sealed capsules, shown in Fig. 3, may be safely handled, will withstand a reasonable amount of rough treatment, and 10 if desired, may be packed and shipped before inserting in the cartridges as shown in Fig. 7.

I claim—

1. A gas cartridge containing "gas", the 15 material of the container comprising a body of gelatin containing glycerine.

2. A gas cartridge containing "gas", the material of the container comprising a body of gelatin containing a quantity of glycerine 20 equal to from about nine percent to about thirty-five percent of the net weight of the gelatin.

3. A gas cartridge containing "gas", the material of the container comprising a body 25 of gelatin containing a quantity of glycerine equal to approximately thirty-three percent of the net weight of the gelatin.

4. A gas cartridge containing "gas", the material of the container comprising a body 30 of one material coated inside with a gelatin composition containing a quantity of glycerine equal to from about nine percent to about thirty-five percent of the net weight of the gelatin.

35 5. A gas cartridge containing "gas", the material of the container comprising a body of non-brittle soft flexible gelatinous material, said gelatinous material containing gelatin and glycerine, and sealed with a molten 40 mass of gelatinous material.

6. The method of making a gas cartridge from non-corrodible gelatin which comprises absorbing a solvent by the gelatin, melting the soaked gelatin, adding glycerine to the melted 45 mass, stirring, and forming containers from the gelatin composition, adding the "gas" and sealing the container.

7. The method of making a gas cartridge from non-corrodible gelatin, which comprises 50 absorbing a solvent by the gelatin at about normal room temperature, melting the soaked gelatin at about one hundred and seventy degrees Fahr., adding glycerine in a quantity of from about one-tenth to about one-third 55 of the weight of the gelatin, stirring to make a uniform mass, and forming containers from said mass, adding the "gas" and sealing the container.

8. The method of making a gas cartridge 60 from non-corrodible leak-proof containers, which comprises coating a container inside with a gelatin mass containing glycerine; providing a coated closure for said container, adding the "gas" and sealing said container 65 with a gelatin-glycerine seal.

9. The method of making a non-corrodible leak-proof "asphyxiating" gas cartridge which comprises making the container and closure of a gelatin-glycerine composition, filling said container with the "asphyxiating" 70 gas chemicals, affixing said closure, and sealing said container with a gelatin-glycerine composition.

10. The method of making a gas-cartridge, which comprises making a container and closure of a gelatin-glycerine composition, filling said container with "asphyxiating" gas chemicals, and sealing said container with the closure by applying a body of molten gelatinous material between a wall of a closure and a part of the wall of the container adjacent said closure. 75 80

In testimony whereof, I hereby affix my signature.

BYRON C. GOSS.

85

90

95

100

105

110

115

120

125

130